

April 20, 1971

G. BLASSE ET AL

3,575,879

BIVALENT EUROPIUM ACTIVATED BARIUM OCTABORATE  
LUMINESCENT MATERIAL

Filed May 9, 1969



fig. 1



fig. 2



fig. 3

INVENTOR.  
GEORGE BLASSE  
JAAP DE VRIES  
BY  
*Frank P. J. J. S. S. S.*  
Agent

# United States Patent Office

3,575,879

Patented Apr. 20, 1971

1

3,575,879

**BIVALENT EUROPIUM ACTIVATED BARIUM OCTABORATE LUMINESCENT MATERIAL**  
George Blasse and Jaap de Vries, Emmasingel, Eindhoven, Netherlands, assignors to U.S. Philips Corporation, New York, N.Y.

Filed May 9, 1969, Ser. No. 823,347  
Claims priority, application Netherlands, May 10, 1968,  
6806648  
Int. Cl. C09k 1/66

U.S. CL. 252—301.4

3 Claims

## ABSTRACT OF THE DISCLOSURE

Bivalent europium activated barium octaborate phosphors, in which the greater part of the luminescent energy is radiated between 380 and 440 nm. in response to ultraviolet exciting radiation, have utility in mercury vapor discharge lamps.

The invention relates to a low-pressure mercury vapour discharge lamp including a luminescent material provided on a support, which luminescent material can be excited by ultraviolet radiation. Furthermore the invention relates to such a material.

In many photochemical document-copying systems a document is copied by irradiating the master and directing the radiation which has been reflected or transmitted to a piece of paper which is sensitive to this radiation and contains substances which can be decomposed by the radiation so that a copy of the master document is obtained possibly after further treatment, for example, fixing.

For efficient use of the reproduction papers it is of course desirable to have a radiation source which emits a strong radiation at those wavelengths to which the paper is most sensitive.

A requirement generally imposed on the reproduction papers to be used is that the substances which are sensitive to radiation are converted as little as possible by normal daylight. This of course facilitates working with these papers and also imposes few requirements on the storage thereof. Since normal daylight contains comparatively little ultraviolet radiation the best combination is apparently a paper which has a maximum sensitivity below 400 nm. and a radiation source which emits a strong ultraviolet radiation.

As already stated above the master to be copied must transmit or reflect the radiation. It has been found that many documents are made from paper which transmits and/or reflects ultraviolet radiation comparatively poorly. In view of the contradictory requirements for document-copying machines a compromise must therefore be made; it is therefore preferred to use light-sensitive papers the maximum sensitivity of which lies between 380 and 440 nm. and a radiation source having a maximum of the emitted radiation between these two values.

Document-copying machines generally use as radiation sources mercury vapour discharge lamps including a luminescent layer provided on a support which layer converts a great part of the ultraviolet radiation produced in the mercury vapour discharge into radiation of longer wavelength. Thus, as described above, the maximum emitted radiation energy must preferably be in the wavelength range between 380 and 440 nm. This is, for example, the case with the very frequently used substance, calcium tungstate. The conversion efficiency of the ultraviolet radiation of the mercury vapour discharge into the radiation between 380 and 440 nm. is, however, comparatively small for this substance, because the emission spectrum is very wide and hence much radiation energy is emitted at wavelengths outside this range. In addition, the absorption spectrum of most light-sensitive papers is con-

2

siderably narrower than this range. As a result of these two causes only a comparatively small part of the total radiation energy emitted by the calcium tungstate is efficiently used by the sensitive paper.

5 A further luminescent substance, which is very frequently used, is a lead-activated silicate of strontium, barium and magnesium. The emission spectrum of this substance is not very wide when excited by the ultraviolet radiation of a mercury vapour discharge, and hence is more suitable for adaptation to the absorption spectrum of a radiation-sensitive paper; the maximum emission of this substance lies, however, at 355 nm. and is therefore less suitable to be transmitted or reflected by the paper of most documents. In spite of this fact the substance is very frequently used on account of the narrow emission band and the strong radiation.

10 A low-pressure mercury vapour discharge lamp according to the invention includes a luminescent material provided on a support and is characterized in that this luminescent material is an alkaline earth borate activated by bivalent europium and having the following composition



wherein

$$0 \leq x+y \leq 0.15$$

$$0 \leq y \leq 0.05$$

$$0.003 \leq p \leq 0.05$$

15 A luminescent material which is represented by the above formula can be excited satisfactorily by ultraviolet radiation which is emitted by a low-pressure mercury vapour discharge lamp and the material then shows an emission spectrum in which the greater part of the luminescent energy is radiated between 380 and 440 nm. Since the conversion efficiency is also very high, namely considerably higher than that of calcium tungstate and approximately as high as that of the above-mentioned silicate, a lamp according to the invention is more suitable for use in document-copying apparatus in combination with available radiation-sensitive types of paper having a maximum absorption within this range, because all requirements as set above are now simultaneously satisfied. In addition it has been found that the substances according to the invention have a good temperature dependence, that is to say, their conversion efficiencies decrease only slightly as the temperature increases. They are thus very suitable for use in high-power low-pressure mercury vapour discharge lamps whose wall temperature assumes a high value during operation.

20 As is evident from the above given formula, a luminescent material according to the invention consists of a barium octaborate activated by bivalent europium wherein the barium may be partly replaced by strontium and/or calcium. In fact, tests have shown that the luminescent properties do not substantially change when replacing small quantities of barium by strontium and/or calcium. Thus, for example, the maximum in the emission spectrum for all materials according to the invention lies at the same wavelength, namely at approximately 400 nm.

25 For contents of strontium and calcium outside the above given limits substances are obtained which are less suitable for practice, because the quantum efficiency and the light output of the luminescent materials then become too small. Pure barium octaborate activated by bivalent europium is preferred.

30 It is to be noted that luminescent materials are known from United States patent specification No. 2,920,046 which have a fundamental lattice according to the formula  $a\text{MeO}_b\text{B}_2\text{O}_3$ , wherein Me is at least one of the metals calcium, strontium, barium and cadmium and wherein the ratio  $a/b$  has a value between  $\frac{1}{2}$  and  $\frac{1}{4}$ . The substances mentioned in the said patent specification are activated by manganese together with lead and/or

bismuth. The known substances do not, however, emit in the blue part, but in the green and yellow parts of the spectrum.

The amount of bivalent europium may be varied between the above-mentioned limits, but is preferably chosen to be between 0.008 and 0.02. In fact, the highest radiation efficiency is found in this range.

In addition to the above-mentioned advantages of the luminescent materials according to the present invention it is to be noted that the substances are only slightly affected by oxidation. This is of great importance in the manufacture of mercury vapour discharge lamps, because they are then often exposed for a short period to a heat treatment in air at a fairly high temperature, for example, 600° C. Such a heat treatment is necessary, for example, when an organic binder is used which is to be removed later on by a heat treatment.

A special advantage of a luminescent material according to the present invention is that a light-reflecting layer of titanium dioxide may fruitfully be used in the mercury vapour discharge lamps according to the invention. The use of such a layer in low-pressure mercury vapour discharge lamps is known. This light-reflecting layer, which is provided between the support of the luminescent material and the luminescent material, very strongly reflects visible radiation emitted by the luminescent material. In this manner it is, for example, possible to manufacture lamps in which the visible radiation from one side of the lamp is accentuated. Such a principle would be very desirable for use in lamps for document-copying apparatus. However, if luminescent materials are used of which the emitted radiation energy lies for a considerable part in the ultraviolet part of the spectrum, for example, the two above-mentioned known substances and particularly the silicate of barium, strontium and magnesium, the use of a titanium dioxide reflector layer is hardly useful because the reflection of titanium dioxide is small for ultraviolet radiation. This applies particularly to the rutile modification of the titanium dioxide; this reflects substantially no radiation below a wavelength of approximately 400 nm. The reflection of the anatase modification extends slightly further, namely down to a wavelength of approximately 380 nm.

In a low-pressure mercury vapour discharge lamp according to the invention a reflecting titanium dioxide layer may be fruitfully used, particularly titanium dioxide in the anatase modification, because at least the greater part of the radiation emitted from the luminescent material is within the reflection range of the titanium dioxide.

Some embodiments of the present invention will now be described with reference to one table, the following example and the accompanying diagrammatic drawing.

A mixture was made of the substances indicated in column III of the table in the quantities indicated in column IV. Since the boric acid partly evaporates during the reaction, an excess of  $H_3BO_3$  of approximately 20% relative to the stoichiometric quantity is always used.

The mixture was heated at approximately 600° C. for 4 hours. After cooling of the firing product obtained it was ground and again heated at approximately 750° C. for 4 hours. In both cases the heat treatment took place in a mixture of nitrogen and hydrogen. The ratio of nitrogen to hydrogen is then not critical; a ratio of, for example, 20:1 was found to be quite usable. The hydrogen serves for reducing the trivalent europium to bivalent europium. After cooling subsequent to the second heat treatment the reaction product obtained was ground and sieved, if necessary. The product was then ready for use.

The quantum efficiency  $q$  is given in column V of the table in percent. The percentages indicated show the conversion efficiencies of the absorbed exciting quanta.

To obtain a measure of the light output of the luminescent materials the quantum efficiency is to be multiplied by the absorption factor. The absorption factor is supposed to be equal to  $1-r$ , wherein  $r$  represents the reflection factor.

The absorption factor is indicated in column VI. The relative light output (r.l.o.) of the luminescent materials as indicated in column VII are then derived from the equation:

$$r.l.o. = q \cdot (1-r)$$

The wavelength of the maximum of the emission band for the different materials was found to be always approximately 400 nm.

All measurements were made using an exciting radiation which had a wavelength of 254 nm.

In the drawing

FIG. 1 diagrammatically shows a low-pressure mercury vapour discharge lamp according to the invention;

FIG. 2 is a graphic representation of the radiation intensity of the substance of Example 2 of the table, and of two known substances, as a function of the wavelength,

FIG. 3 is a graphic representation of the variation of the radiation intensity of the substance of Example 2 with temperature.

FIG. 1 shows a low-pressure mercury vapour discharge lamp which includes an envelope 1. Electrodes 2 and 3, between which the discharge takes place during operation of the lamp, are provided at the ends of the lamp. The inner side of the envelope 1 which is made of, for example, glass, is coated with a luminescent layer 4 which contains a luminescent material according to the present invention. The luminescent substance is provided on the envelope 1 in any conventional manner.

| I       | II                                              | III                                       | IV    | V  | VI   | VII    |
|---------|-------------------------------------------------|-------------------------------------------|-------|----|------|--------|
| Example | Formula                                         | Composition<br>firing mixture<br>in grams |       | q  | 1-r  | r.l.o. |
| 1.....  | $Ba_{0.99}Eu_{0.005}B_3O_{13}$                  | $BaCO_3$                                  | 1.970 |    |      |        |
|         |                                                 | $Eu_2O_3$                                 | 0.009 | 60 | 0.60 | 36     |
|         |                                                 | $H_3BO_3$                                 | 6.000 |    |      |        |
| 2.....  | $Ba_{0.99}Eu_{0.01}B_3O_{13}$                   | $BaCO_3$                                  | 1.960 |    |      |        |
|         |                                                 | $Eu_2O_3$                                 | 0.018 | 60 | 0.70 | 42     |
|         |                                                 | $H_3BO_3$                                 | 6.000 |    |      |        |
| 3.....  | $Ba_{0.98}Eu_{0.02}B_3O_{13}$                   | $BaCO_3$                                  | 1.940 |    |      |        |
|         |                                                 | $Eu_2O_3$                                 | 0.036 | 45 | 0.85 | 38     |
|         |                                                 | $H_3BO_3$                                 | 6.000 |    |      |        |
| 4.....  | $Ba_{0.89}Sr_{0.10}Eu_{0.01}B_3O_{13}$          | $BaCO_3$                                  | 1.760 |    |      |        |
|         |                                                 | $SrCO_3$                                  | 0.147 |    |      |        |
|         |                                                 | $Eu_2O_3$                                 | 0.018 | 45 | 0.75 | 34     |
|         |                                                 | $H_3BO_3$                                 | 6.000 |    |      |        |
| 5.....  | $Ba_{0.84}Sr_{0.15}Eu_{0.01}B_3O_{13}$          | $BaCO_3$                                  | 1.660 |    |      |        |
|         |                                                 | $SrCO_3$                                  | 0.220 |    |      |        |
|         |                                                 | $Eu_2O_3$                                 | 0.018 | 40 | 0.75 | 30     |
|         |                                                 | $H_3BO_3$                                 | 6.000 |    |      |        |
| 6.....  | $Ba_{0.94}Ca_{0.05}Eu_{0.01}B_3O_{13}$          | $BaCO_3$                                  | 1.860 |    |      |        |
|         |                                                 | $CaCO_3$                                  | 0.050 |    |      |        |
|         |                                                 | $Eu_2O_3$                                 | 0.018 | 40 | 0.75 | 30     |
|         |                                                 | $H_3BO_3$                                 | 6.000 |    |      |        |
| 7.....  | $Ba_{0.89}Sr_{0.05}Ca_{0.05}Eu_{0.01}B_3O_{13}$ | $BaCO_3$                                  | 1.760 |    |      |        |
|         |                                                 | $SrCO_3$                                  | 0.074 |    |      |        |
|         |                                                 | $CaCO_3$                                  | 0.050 |    |      |        |
|         |                                                 | $Eu_2O_3$                                 | 0.018 | 40 | 0.75 | 30     |
|         |                                                 | $H_3BO_3$                                 | 6.000 |    |      |        |

The broken-line curve **a** in the graph of FIG. 2 shows the spectral energy distribution of the known lead-activated silicate of barium, strontium and magnesium and the broken-line curve **b** shows the spectral energy distribution of the known calcium tungstate. These curves are shown for comparison both for the spectral distribution and for the intensity of the luminescent radiation. The maximum intensity of the curve **a** is fixed at 100. The curve **2** relates to the material of Example 2 of the table. As is clearly evident from the drawing, luminescent materials which are used in lamps according to the present invention have a more favourable location of the maximum emission in the spectrum as compared with the known silicate, while they have considerably higher peak values and a narrower emission range as compared with the known calcium tungstate.

The curve **2** in the graph of FIG. 3 shows the temperature dependence of the radiation intensity of the material of Example 2. The temperature is plotted in °C. on the abscissa. The maximum intensity is fixed at 100. The figure shows that the borates according to the invention have a very good temperature dependence and still show an intensity of the luminescent radiation at approximately 220° C. which is equal to half the maximum value. It may be noted for comparison that already at 75° C. the intensity of the known calcium tungstate has decreased to half the value at room temperature.

While we have described our invention in connection with specific embodiments and applications, other modifications thereof will be readily apparent to those skilled

in this art without departing from the spirit and scope of the invention as defined in the appended claims.

What we claim is:

1. An alkaline earth borate luminescent material activated by bivalent europium and having the composition



wherein

$$0 \leq x+y \leq 0.15$$

$$0 \leq y \leq 0.05$$

$$0.003 \leq p \leq 0.05$$

2. The luminescent material of claim 1 which material has the composition



wherein  $0.003 \leq p \leq 0.05$ .

3. The luminescent material of claim 1 wherein  $0.008 \leq p \leq 0.02$ .

#### References Cited

##### UNITED STATES PATENTS

|           |        |                       |           |
|-----------|--------|-----------------------|-----------|
| 3,423,325 | 1/1969 | Wanmaker et al. ----- | 252—301.4 |
| 3,431,216 | 3/1969 | Chenot -----          | 252—301.4 |

##### FOREIGN PATENTS

|         |        |                   |           |
|---------|--------|-------------------|-----------|
| 6408082 | 1/1966 | Netherlands ----- | 252—301.4 |
|---------|--------|-------------------|-----------|

TOBIAS E. LEVOW, Primary Examiner

R. D. EDMONDS, Assistant Examiner